

## UNITED STATES PATENT OFFICE

2,640,806

## PROCESS FOR POLISHING ALUMINUM

Frederick Harold Hesch, Spokane, Wash., assignor to Kaiser Aluminum & Chemical Corporation, a corporation of Delaware

No Drawing Application June 27, 1949,  
Serial No. 101,693

7 Claims. (Cl. 204—140.5)

1

This invention relates to the brightening of aluminum and aluminum alloys. More particularly, the invention relates to a composition and method for chemical brightening of aluminum and its alloys.

Although aluminum is ordinarily considered a bright metal, it often presents a dull or matte-like finish due to the oxide films formed on its surfaces during processing. Many aluminum and aluminum alloy products are fabricated from mill finished sheet having such a characteristic dull appearance, which leads to a demand by fabricators for means to impart a bright, lustrous finish to their products. One widely used method of polishing aluminum and its alloys is by mechanical buffing with a suitable abrasive. However, this mechanical polishing is expensive and is not easily adaptable to articles having intricate shapes and inaccessible surfaces. Other methods known as electropolishing and electro-brightening involve subjecting the aluminum article to an electrolytic treatment and producing desirable lustrous finishes. However, these methods are both slow and expensive.

It is therefore, a primary object and purpose of the invention to provide a composition and method for the chemical brightening or polishing of aluminum. A further object is to provide a chemical solution or bright dip composition for aluminum and aluminum alloys which is characterized by its economy in use, short immersion time required to obtain the desired effect, and an ease of application. Another object is to produce of aluminum and aluminum alloy articles polished or brightened surfaces by means of a chemical bright dip composition and process which effectively removes the dulling oxide films from the metallic surfaces and imparts thereto a high luster.

Chemical brightening of aluminum has previously been accomplished using a combination of nitric and hydrofluoric acids. The hydrofluoric acid readily dissolves any oxide film and attacks the metal. The nitric acid, which is essentially inactive toward aluminum, serves to dissolve any metallic smut which might deposit out of solution onto the metal surface being treated. However, the etching action of the HF proved difficult to control regardless of the concentration or temperature employed, and uniform results could not be consistently obtained.

It has been discovered according to the present invention that if a noble metal, such as gold, palladium or platinum, is used as an electrode and is electrically connected to the aluminum or alloy article immersed in the solution of nitric

and hydrofluoric acids, a superior brightening of the surfaces of the article is obtained. The term "noble metal" as used in the specification and claims is intended to include gold, platinum and palladium.

Platinum, palladium and gold being at the extreme end of the electromotive force series are impervious to attack by the acidic constituents of the bath. In addition, they form with aluminum, a galvanic cell or couple having a high electric potential. It is believed that this fact accounts for the greatly enhanced brightening effect. It is only necessary in forming the couple that these noble metal electrodes and the aluminum or aluminum alloy be electrically connected either within the cell or externally. Without this couple, the solution forms an etched or frosted finish; but when the "noble" metal electrode is connected to the aluminum and the couple is formed, a bright finish is obtained. Gold and platinum are the preferred electrode materials.

The aluminum article is connected or joined to the noble metal, which latter may be in the form of strips or of a bath container lining or inner jacket. The electrode and the work may be electrically connected, for example, outside the cell by means of a wire, or within the cell by direct contact. The electrode area is preferably approximately that of the area of the work piece although good results are obtained where the electrode area is not directly related to the area of the work piece.

While the combination of nitric acid, hydrofluoric acid and metallic gold or platinum produce bright surfaces, it was found that addition of a mild inhibitor such as glycerine would improve the brightness. Any of the lower molecular weight polyhydric aliphatic alcohols, such as ethylene glycol, diethylene glycol, propylene glycol, mannitol, and sorbitol are also suitable as inhibitors.

The amounts of nitric and hydrofluoric acids, and polyhydric alcohol used are preferably within the following ranges:

| Constituent        | Volume Concentration, cc./liter | Percent Weight of Solution |
|--------------------|---------------------------------|----------------------------|
| HNO <sub>3</sub>   | 5-60 (70% HNO <sub>3</sub> )    | 5-6                        |
| HF                 | 2-9 (48% HF)                    | 01-.5                      |
| Polyhydric Alcohol |                                 | 5-5                        |
| Water—Balance      |                                 |                            |

The fluoride ion is preferably introduced in the form of hydrofluoric acid, although any suit-

able soluble salt of the acid which will form hydrofluoric acid in situ in the solution in the presence of nitric acid may be used, for example, ammonium fluoride.

The fluoride ion concentration should be maintained at a value corresponding to that produced by amounts of hydrofluoric acid within the above-stated range.

The proper hydrogen ion concentration is primarily maintained by the use of nitric acid in an amount within the above indicated range.

Thus, the bright dip composition of the present invention comprises an aqueous acid solution containing hydrogen, nitrate, and fluoride ions in concentration corresponding to that produced by a solution containing from about .5 to about 6% nitric acid, and from about .01 to about 0.5% hydrofluoric acid by weight for use in conjunction with noble metal electrodes electrically connected to the aluminum or aluminum alloy work piece. In addition, the solution preferably contains from about .5 to about 5% by weight of a lower molecular weight polyhydric aliphatic alcohol.

Excellent brightening results are obtained when the hydrogen and fluoride ion concentrations are maintained at any combination of values corresponding to that produced by a solution containing nitric acid and hydrofluoric acid, and preferably a polyhydric alcohol inhibitor, in any combination of constituent amounts within the ranges set forth above, or any combination of equivalent substances which will produce a solution of substantially the same chemical composition.

It is to be noted that a satisfactory degree of brightening is obtained when using any of the constituents in slightly smaller or larger amounts than indicated above. However, the desired effect is more readily obtained by operating within the stated ranges.

The chemical bath may be operated at temperatures of from about 100° F. to the boiling point. The desired brightening is accomplished with a shorter immersion time at the higher temperatures of from about 190° F. to boiling, and accordingly, this range is preferred. The time of immersion of the articles being treated in the bath should be sufficient to produce the desired brightening, yet insufficient to cause any undue etching of the metal. It is, of course, dependent primarily on solution temperatures and concentrations and may be widely varied. An immersion time of from about one-half to about ten minutes is most desirable.

The following example of a chemical dip solution producing maximum brightness is illustrative of a specific embodiment, and is not to be construed as a limitation of the invention:

| Constituent            | Volume Concentration, c.c./liter | Percent Weight of Solution |
|------------------------|----------------------------------|----------------------------|
| HNO <sub>3</sub> ..... | 50 (70% HNO <sub>3</sub> ).....  | 5                          |
| HF.....                | 2 (48% HF).....                  | 1                          |
| Glycerol.....          | 25.....                          | 3                          |
| Water-Balance.....     | .....                            | .....                      |

A gold strip electrode was electrically connected to the work piece to be brightened during immersion of the latter in the solution.

The procedure followed in treating the metal articles with the chemical bath is merely to establish electrical connection between the work piece and the platinum or gold electrode and then immerse the article in the heated solution

for the required time and thereafter thoroughly water rinse and dry the treated article. However, it is advantageous that the metal to be processed be cleaned or degreased by the use of a mild, inhibited alkaline cleaner. This is preferably accomplished by immersion in a heated solution of the cleaner for a few minutes, for example, two minutes in solution at 180°-200° F., followed by a thorough rinsing prior to introduction into the bright dip solution.

Agitation of the bath is not essential, but is recommended since it produces more uniform results and tends to decrease the required immersion time. Mechanical or air agitation may be used, but the former is preferable since it does not cool the solution as does air agitation.

The process may be operated on a continuous or semicontinuous basis, or it may be conducted as a batch process. In case of the former, the components are gradually depleted and calculated additions are periodically added to maintain proper concentrations.

The chemical polishing treatment may be conducted in any suitable tank or other apparatus provided with a lining impervious to the corrosive action of the nitric and hydrofluoric acids at the operating temperatures. A particularly useful lining is Karbate—a treated carbon product resistant to attack by all chemicals except those which are highly oxidizing. Karbate is manufactured in molded slabs, blocks and other shapes.

The heating of the solution may be accomplished by the use of Karbate tubes or heat exchangers, or, if electrical heating is desired Karbate shielded immersion heaters may be employed.

The results obtained with the chemical bright dip of the present invention do not produce a surface smoothing effect in comparison to mechanical buffing or electropolishing. However, the surface luster or brightness compares very favorably with that produced by electrobrightening, while the chemical bright dip requires only a short immersion time and no electric current. In short, the improved chemical bath produces the desired result much more economically.

What is claimed is:

1. A process for the chemical brightening of aluminum and aluminum alloys which comprises electrically connecting the work to a noble metal electrode, and subjecting the work to the action of an aqueous acid solution consisting essentially of hydrogen, nitrate and fluoride ions in concentration corresponding to that produced by a solution containing from about .5 to 6% nitric acid, and about .01 to 0.5% hydrofluoric acid by weight, and maintaining the solution at a temperature of from about 100° F. to the boiling point.

2. A process for the chemical brightening of aluminum and aluminum alloys which comprises forming a galvanic couple between the work and a noble metal electrode in an aqueous acid solution consisting essentially of from about .5 to 6% nitric acid and about .01 to 0.5% hydrofluoric acid by weight, and maintaining the solution at a temperature of from about 100° F. to the boiling point for a time sufficient to brighten the work.

3. A process according to claim 1 in which the solution contains from about .5 to 5% of a lower molecular weight polyhydric aliphatic alcohol as an inhibitor.

4. A process according to claim 2 in which the

solution contains from about .5 to 5% of a lower molecular weight polyhydric aliphatic alcohol as an inhibitor.

5. A process according to claim 2 in which the noble metal electrode is gold.

6. A process according to claim 2 in which the noble metal electrode is platinum.

7. A process for the chemical brightening of aluminum and aluminum alloys which comprises treating the metal with an acid aqueous solution consisting essentially of from about .5 to 6% nitric acid, about .01 to 0.5% hydrofluoric acid, and about .5 to 5% glycerol by weight of solution in the presence of a noble metal electrode, said electrode being electrically connected to the metal work, maintaining the solution at a temperature of from about 190° F. to the boiling

point, withdrawing and rinsing the work after an immersion of from about one-half to about ten minutes.

FREDERICK HAROLD HESCH.

References Cited in the file of this patent

UNITED STATES PATENTS

|    | Number    | Name     | Date          |
|----|-----------|----------|---------------|
| 10 | 2,037,633 | Kelvie   | Apr. 14, 1936 |
|    | 2,052,962 | Booe     | Sept. 1, 1936 |
|    | 2,375,394 | Tosterud | May 8, 1945   |

FOREIGN PATENTS

|    | Number  | Country | Date          |
|----|---------|---------|---------------|
| 15 | 798,721 | France  | Mar. 11, 1936 |
|    | 471,053 | Germany | Feb. 6, 1929  |